

3,338,829

**CORROSION-INHIBITED AMMONIUM ORTHOPHOSPHATE SOLUTIONS AND COMPOSITIONS  
USEFUL FOR MANUFACTURING THEM**  
Robert P. Langguth, St. Louis, and William W. Morgenthaler, Bridgeton, Mo., assignors to Monsanto Company, St. Louis, Mo., a corporation of Delaware  
No Drawing. Filed May 6, 1964, Ser. No. 365,492  
10 Claims. (Cl. 252—2)

This invention relates to improved aqueous solutions of phosphate salts, which solutions are characterized by having a significantly reduced tendency to corrode copper metal and copper-containing alloys. More specifically, the present invention relates to corrosion-inhibited ammonium phosphate solutions suitable for prolonged use in handling and storage equipment made of copper and/or copper alloys and to the compositions useful for manufacturing them.

Aqueous ammonium phosphate solutions have many uses: One of the most valuable recent developments in the field of fire fighting, and more particularly, forest fire fighting, was that relating to the use of aqueous solutions of ammonium phosphate salts. Since the present invention is particularly valuable when practiced in connection with forest fire fighting, the present discussion will be directed toward this particular end use. However, it should be kept in mind that the invention is generally useful for inhibiting corrosion of copper by ammonium phosphate solutions. Ordinarily, the solutions (often thickened with a viscosity modifying agent so that the solutions stick readily to surfaces with which they come into contact) are dropped by airplanes such as air-tankers onto brush, trees and dry grass in the path of a fire in order to slow or stop the progress of the fire. The extensive use of such ammonium phosphate solutions for forest fire control has been slowed because of the concern by those in the field over the natural corrosivity of such aqueous ammonium phosphate solutions toward some of the vital parts of air-tankers and storage equipment.

Aqueous solutions containing several weight percent of dissolved ammonium phosphate are considered to be corrosive toward copper metal or copper alloys such as brass and bronze and the like, and such are corrosive to the extent to cause great concern when the aqueous solutions are to come into physical contact with vital aircraft parts, since failure of the aircraft parts due even to slow corrosion occurring over a prolonged period of time could result in the loss of the aircraft and crew. Thus, in order to be considered completely acceptable for use in forest fire fighting by the air-drop method, it is necessary that the corrosivity of aqueous ammonium phosphate solutions, particularly toward copper metals, be significantly reduced.

Consequently, it is an object of the present invention to provide aqueous solutions containing ammonium phosphate salts useful for forest fire fighting, the normal tendency of which to corrode copper and copper-containing alloys is significantly reduced or substantially eliminated.

It is another object of the present invention to provide novel methods of inhibiting the corrosion of copper equipment by aqueous ammonium phosphate solutions.

It is a still further object of the present invention to provide ammonium phosphate compositions which are useful in preparing aqueous ammonium phosphate solutions characterized by having a significantly reduced tendency to corrode copper metal and copper-containing alloys.

It has now been found that the normal or natural tendency of aqueous solutions of ammonium phosphate

salts, such as, for example, monoammonium orthophosphate and diammonium orthophosphate to corrode copper equipment can be significantly reduced and even practically eliminated by the presence (in solution) of an effective amount of an inorganic water-soluble iodide compound. The term "inorganic water-soluble iodide" is intended to include all of those inorganic iodide materials or compounds that are soluble in the ammonium phosphate solutions in which they are to be utilized to the extent of at least about 0.005 weight percent. It includes, for example, the alkali metal and alkaline earth metal iodides such as sodium, potassium, lithium, calcium, magnesium and strontium iodides as well as ammonium iodide. Of these, generally sodium, potassium and/or ammonium iodides are preferred. In addition, other water soluble inorganic iodide compounds include iodine, hydrogen iodide, and the iodide compounds of the polyhalide complex salts, such as the halides of alkali metals and other strong bases which include  $RbI_3$ ,  $(C_6H_5)_2H_3$ ,  $N(CH_3)_4I_2$ ,  $N(C_2H_5)_4IBr_2$ ,  $KIBrCl$ ,  $KICl_4$ ,  $KIF_4$ , and the like. Actually, since the protection from corrosion that can be afforded copper equipment by practicing the present invention apparently results from the iodide (anion) portion of the iodide compound, the particular source from which the iodide anions are derived in manufacturing the aqueous ammonium phosphate solutions is not at all critical, provided a sufficient amount of iodide anions are provided in the phosphate solutions to effectively decrease the normal corrosivity of the phosphate solutions toward copper and copper-containing alloys.

The inorganic iodide compounds are effective in aqueous solutions of ammonium phosphates of normally useful concentrations and which in most cases are from about 0.5 weight percent and up to the level at about 35 which the solutions are saturated therewith, of dissolved ammonium phosphate salts, including monoammonium orthophosphate and/or diammonium orthophosphate salts, and also including the diammonium and monoammonium mixed orthophosphate salts that also contain 40 an alkali metal cation, such as monoammonium disodium orthophosphate, monoammonium dipotassium orthophosphate and the like, no matter from what source these materials were derived, or in what form the materials are initially introduced into the aqueous compositions. Especially preferred aqueous ammonium phosphate compositions contain from about 5 to about 25 weight percent of an ammonium orthophosphate. Generally, it is preferred that the inhibited aqueous phosphate solutions of this invention have a pH between about 3 and 50 about 9. When monoammonium orthophosphate is the only ammonium phosphate salt present in the inhibited fire-control compositions of this invention, the preferred pH of these compositions is generally from about 3 to about 5. Similarly, when diammonium orthophosphate is the only ammonium phosphate salt contained therein, the preferred pH is from about 7 to 9. When mixtures of monoammonium orthophosphate and diammonium orthophosphate are utilized, pH's between these preferred ranges are generally more desirable. However, compositions having pH's somewhat higher or lower than these preferred ranges can also be utilized to advantage in the practice of the present invention.

Although the presence of even a very small amount of the water-soluble iodide compounds in the aqueous ammonium phosphate solutions described above has a corrosion-inhibiting effect upon them, as a general rule, aqueous phosphate compositions containing from about 0.01 to about 10 and even higher amounts can be used although such does not appear to appreciably improve 65 the corrosion inhibition of the aqueous ammonium phosphate solutions over the use of lesser amounts. Preferably from about 0.10 to about 4 weight percent of one

or more of the iodide compounds in the dissolved state should be utilized.

The corrosion-inhibited ammonium phosphate solutions of the present invention can also contain materials other than the phosphate salts and the iodide compounds without detracting substantially from the benefits that can be obtained by practicing this invention, for example, the solutions can contain minor amounts of surfactants; inorganic and organic complexing agents such as the alkali metal tripolyphosphate, pyrophosphates and trimetaphosphates, as well as the higher polyphosphates such as the hexametaphosphates and also can contain ethylenediamine tetraacetic acid and various alkali metal and ammonium salts thereof and the alkali metal and ammonium nitrilotriacetates; any of the various thickening agents such as carboxymethylcellulose, algin, clays such as bentonites and attapulgites and the like, guar gum, pectates such as lemon pectates, and the like, and carboxyethylcellulose; other corrosion-inhibiting ingredients; and inorganic and organic pigments and dyes; as well as many other materials.

A particular advantage in the use of the inorganic water-soluble iodide compounds in ammonium phosphate solutions is that they are particularly effective in the presence of water soluble fluosilicates compounds such as sodium fluosilicate, ammonium fluosilicate and potassium fluosilicate, which are useful as inhibitors for aluminum in contact with ammonium phosphate solutions and therefore provide ammonium phosphate solutions which are characterized by having a significantly reduced tendency to corrode not only copper-containing metals but also aluminum-containing metals. In fact, in most cases, the combination of the iodide compounds and the fluosilicate compounds function better as corrosion inhibitors for copper and copper-containing alloys than the iodide compound when used individually. Such fluosilicates are described and disclosed in U.S. Re. 25,394.

The corrosion-inhibited phosphate compositions of this invention can be manufactured via any of a number of manipulative methods without any noticeably detrimental effects upon the ultimate performance of the compositions. For example, the iodide compound can simply be dissolved by intermixing it into or with the otherwise completely formulated aqueous compositions, or at any other stage during the preparation of the fire-control composition. Via another method, the iodide compound can first be dissolved in water, and the resulting solution then intermixed subsequently with the ammonium phosphate materials.

Still another process for manufacturing the aqueous corrosion-inhibited phosphate compositions described heretofore involves one of the preferred embodiments of the present invention. This preferred embodiment comprises a "concentrate" mixture of one or more of the ammonium phosphate salts described heretofore with one or more of the iodide (inhibitor) compounds, generally in a particulated, solid form. Preferably the inhibitor compound(s) and ammonium phosphate salt(s) will be present in this concentrate composition or mixture in amounts proportionate to those found in the fire-control compositions described heretofore, so that the final fire-control composition can be manufactured by simply dissolving the concentrate in a sufficient amount of water. In other words, generally the preferred concentrate compositions of this invention will contain at least one of the above-described ammonium phosphate salts and at least one of the iodide (inhibitor) compounds in a weight ratio of phosphate salt to inhibitor compound, respectively, of from about 4,000:1 to about 1:1, and preferably from about 400:1 to about 2.5:1. These preferred concentrate compositions can also contain effective amounts of practically any other ingredients, including a thickener if one is desired in the final fire-control compositions, as well as dyes, pigments, water-softening agents and the like, all of which should preferably be present in the concentrate

compositions in minor amounts, as compared to the ammonium phosphate salt(s) contained therein. Especially preferred concentrate compositions contain a major amount of the ammonium orthophosphate material, that is, at least about 50 weight percent, in addition to the minor amounts, that is, less than 50 weight percent, of the corrosion inhibitor, thickener, and other desired additives. Some of the advantages of these preferred concentrate compositions can readily be appreciated when it is realized that at most points from which aircraft are loaded for their various air-drops of fire-control compositions, very little weighing and handling equipment is available that is capable of manufacturing the fire-control compositions from the individual components. Thus, in the absence of the preferred concentrate compositions described above (which concentrate compositions need simply be dissolved in appropriate amount of water in order to be converted into the final valuable fire-control compositions of the present invention), as a practical matter, such corrosion inhibited final fire-control compositions as those described heretofore could not be utilized.

Typical examples of the preferred concentrate compositions of this invention include:

- (a) 99.0 weight percent of diammonium orthophosphate and 1.0 weight percent of potassium iodide.
- (b) 90.0 weight percent of monoammonium orthophosphate, 1.0 weight percent of ammonium iodide and 9.0 weight percent of sodium alginate.
- (c) 90 weight percent of diammonium orthophosphate, 0.5 weight percent of sodium iodide and 9.5 weight percent of sodium carboxymethylcellulose.
- (d) 55 weight percent of an equimolar mixture of monoammonium orthophosphate and diammonium orthophosphate, 1.0 weight percent of ammonium iodide, 35 weight percent of sodium tripolyphosphate and 9 weight percent of sodium alginate.
- (e) 89 weight percent of monoammonium orthophosphate, 0.25 weight percent of magnesium iodide and 10.75 weight percent of pentasodium aminotrimethylenephosphonate.
- (f) 70 weight percent of diammonium orthophosphate, 20 weight percent of monoammonium orthophosphate, 9 weight percent of sodium carboxyethylcellulose and 1 weight percent of potassium iodide.
- (g) 84 weight percent of diammonium orthophosphate, 15.50 weight percent of guar gum and 0.50 weight percent of ammonium iodide.
- (h) 90 weight percent of diammonium orthophosphate, 8 weight percent of sodium carboxymethylcellulose, 1 weight percent of potassium iodide and 1 weight percent of sodium fluosilicate.

These "concentrate" compositions are also useful as corrosion-inhibited de-icer compositions, wherein either alone or in combination with additional corrosion-inhibiting materials, they can be utilized in a manner similar to that in which more corrosive, less desirable sodium chloride is presently conventionally utilized. For example, these particulated, solid ammonium phosphate-iodide compositions can effectively de-ice sidewalks, roadways and the like when they are simply spread over ice and/or snow on these substrates.

The concentrate compositions can be prepared via any of a number of convenient procedures, including simply blending or mixing together the appropriate amounts of the various dry ingredients. Although the size of the individual particles in these preferred concentrate compositions is not critical insofar as the practice of the present invention is concerned, it is generally preferred that they be of sufficiently small size to pass through a U.S. standard 12 mesh screen. For optimum results, at least about 80 weight percent of these particles should be small enough to pass through a U.S. Standard 40 mesh screen.

Although commercial grades of phosphate salts do not necessarily meet these optimum standards of particle

size, they can readily be utilized in the preparation of the compositions of this invention.

In the following example, which is illustrative of one of the preferred embodiments of the present invention, all parts given are by weight unless otherwise specified.

*Example*

Into a conventional iron storage tank fitted with a fairly efficient mixer are charged 89 parts of water and 11.25 parts of a pre-prepared blend made up of 10 parts of crystalline technical grade diammonium orthophosphate, 1 part of carboxymethylcellulose and 0.25 part of potassium iodide. The resulting mixture is then stirred until all of the diammonium orthophosphate has dissolved.

Into the resulting fire-control composition are immersed several clean, preweighed soft copper (1" x 2" x  $\frac{1}{16}$ ") coupons. The coupons are immersed in the composition for a total of 72 hours, after which the coupons are removed from the fire-control composition, rinsed with distilled water and acetone and then reweighed. The loss in weight (in milligrams) is then appropriately inserted into the equation:

$$\frac{534W}{DAT} = \text{Corrision in mils per year}$$

wherein:

W=weight lost during test in milligrams,

D=specific gravity of metal,

A=exposed surface area in square inches,

T=time of exposure to solution in hours,

in order to determine the corrosion that has taken place, expressed in terms of mils of penetration per year. The corrosion rate or rate of attack on copper by the composition of this example is thus found to be about 57 mils per year. When 0.15 part of sodium fluosilicate is added to the foregoing composition, the corrosion rate on copper by the composition of this example is found to be about 4.7 mils.

By comparison, a composition which is prepared in the same way as that in this example, but without the potassium iodide or sodium fluosilicate, corrodes similar copper coupons at a rate of about 1,000 mils per year.

Good results comparable to the foregoing example can also be obtained using substantially equivalent amounts of other iodide compounds which include, sodium iodide, lithium iodide, calcium iodide, magnesium iodide, strontium iodide and ammonium iodide as well as substantially equivalent amounts of various thickening agents which include clays, algin, guar gum, pectates, carboxymethylcellulose and the like.

As being illustrative of an airplane attachment for extinguishing fires as well as the method for using such, reference is made to U.S. Patent 1,997,669.

What is claimed is:

1. An aqueous ammonium orthophosphate composition consisting essentially of, in addition to the ammonium orthophosphate dissolved therein in an amount of at least about 0.5 weight percent of said composition, a water soluble inorganic iodide compound in an amount of at least about 0.01 weight percent of said composition to effectively decrease the normal corrosivity of said composition toward copper and copper-containing alloys.

2. A corrosion-inhibited aqueous ammonium orthophosphate composition as in claim 1, wherein said water-soluble inorganic iodide compound is selected from the group consisting of ammonium, alkali metal and alkaline earth metal iodides.

3. A corrosion-inhibited aqueous ammonium orthophosphate composition as in claim 2, wherein said ammonium orthophosphate salt is selected from the group

consisting of monoammonium orthophosphate, diammonium orthophosphate and mixtures thereof.

4. A corrosion-inhibited aqueous ammonium orthophosphate composition as in claim 3, wherein said ammonium orthophosphate is in an amount of from about 5 to about 25 weight percent and said iodide compound is in an amount of from about 0.10 to about 10 weight percent.

5. A corrosion-inhibited aqueous ammonium orthophosphate composition as in claim 4, additionally containing an effective corrosion-inhibiting amount of a water soluble fluosilicate compound selected from the group consisting of sodium fluosilicate, potassium fluosilicate and ammonium fluosilicate.

10 15 6. A process for inhibiting the corrosion of copper and copper alloys caused by aqueous ammonium orthophosphate solutions containing at least about 0.5 weight percent of an ammonium orthophosphate, which process comprises the dissolution into said solutions of a water-soluble inorganic iodide compound in an amount of at least about 0.01 weight percent.

20 25 7. A concentrated ammonium orthophosphate composition suitable for use in the manufacture of aqueous copper corrosion-inhibited ammonium orthophosphate fire-fighting solutions, said composition consisting essentially of a water-soluble inorganic iodide compound capable of being dissolved in said fire-fighting solution and a major portion of at least one ammonium orthophosphate salt; the weight ratio of said ammonium orthophosphate salt to said iodide compound in said composition being from about 4,000:1 to about 1:1.

30 35 8. A particulated, solid concentrate composition consisting essentially of at least about 50 weight percent of an ammonium orthophosphate material selected from the group consisting of monoammonium orthophosphate, diammonium orthophosphate and mixtures thereof, and, as a copper corrosion inhibitor, an inorganic iodide compound selected from the group consisting of ammonium, alkali metal and alkaline earth metal iodides; the weight ratio of said ammonium orthophosphate material to said iodide compound in said concentrate composition being from about 400:1 to about 2.5:1.

40 45 9. A particulated, solid concentrate composition as in claim 8, wherein said iodide compound is potassium iodide.

10. A method of retarding the corrosion of copper and copper-containing alloys upon contact with a normally corrosive aqueous ammonium orthophosphate solution, which method comprises effecting said contact when said aqueous ammonium orthophosphate in an amount of at least about 0.5 weight percent and contains dissolved therein a water soluble inorganic iodide compound in an amount of at least about 0.01 weight percent.

**References Cited**

**UNITED STATES PATENTS**

|            |         |           |           |
|------------|---------|-----------|-----------|
| Re. 25,394 | 6/1963  | Martinson | 71-34 X   |
| 1,997,669  | 4/1935  | Arcieri   | 169-2     |
| 2,152,659  | 4/1939  | Nitti     | 252-387 X |
| 2,567,156  | 9/1951  | Malowan   | 252-389 X |
| 3,161,598  | 12/1964 | Geld      | 252-387 X |
| 3,223,649  | 12/1965 | Langguth  | 252-146 X |
| 3,249,547  | 5/1966  | Fisher    | 252-389 X |

**OTHER REFERENCES**

Chemical Week, vol. 89, No. 14, Oct. 7, 1961, pp. 39-40.